

B. A. RUGG.  
ROADWAY OR PAVEMENT AND METHOD OF CONSTRUCTING SAME.  
APPLICATION FILED APR. 26, 1917.  
**L,330,139.**

Patented Feb. 10, 1920.

*Fig. 1.*



*Fig. 2.*



*Inventor:*  
Burrard A. Rugg  
*By his Atty's:*  
A. L. Davis, George R. Keen.

# UNITED STATES PATENT OFFICE.

BERNARD A. RUGE, OF TARRYTOWN, NEW YORK, ASSIGNOR TO WARD CARPENTER AND COMPANY, INC., A CORPORATION OF NEW YORK.

## ROADWAY OR PAVEMENT AND METHOD OF CONSTRUCTING SAME.

1,330,139.

Specification of Letters Patent.

Patented Feb. 10, 1920.

Application filed April 26, 1917. Serial No. 164,790.

To all whom it may concern:

Be it known that I, BERNARD A. RUGE, a citizen of the United States, residing at Tarrytown, county of Westchester, and State 5 of New York, have invented certain new and useful Improvements in Roadways or Pavements and Methods of Constructing Same, fully described and represented in the following specification and the accompanying 10 drawings, forming a part of the same.

This invention relates to certain improvements in roadways or pavements particularly adapted for automobiles and other heavy vehicle traffic, and method of 15 constructing the same.

It is the especial object of the invention to provide a road construction which shall be very much cheaper, because of the material used, than prior constructions, and 20 which, because of the materials and the method of laying them, will be durable and will stand up for long periods under the heavy traffic to which roadways are now subjected, particularly by the automobile, 25 the construction being such that, except under unusual conditions, as swampy ground, no special foundation is required, the materials of the road being laid directly on the usual subgrade of dirt or soil.

In modern road constructions, it has been the opinion of road engineers that the road ballast which is used with a binder should have the highest crushing strength, that is, offer the highest resistance to impact shocks. 5 So, when obtainable, trap rock has been used which has such properties, many stones of less crushing strength being rejected as unfit. Trap rock, and for that matter most stone at all suitable for road making, is expensive, but has been considered essential.

I have discovered that coal cinder and similar material, which it is exceedingly desirable to use because of its abundance and cheapness, may, contrary to the usual belief of road engineers, be employed for road ballast in a substantially pure state, that is to say, without mixing it with other ballast material such as trap rock or softer stone or pebbles.

In road constructions where such cinder has been used, the percentage of the cinder has been very small, it having been used, not as the ballast, but mixed with trap rock, broken stone or pebbles, and simply used as a filler between the rock interstices.

I have found by experiment that the use of a substantially pure cinder combined in various ways with a bituminous binder will produce a road bed which will stand up for long periods and which is very much cheaper 60 to construct than road beds employing trap rock or other broken stone or pebbles. This durability of a road constructed of a substantially pure cinder united with a binder and compacted, I attribute possibly to the 65 elasticity of the material which, apparently, yields somewhat, or offers an elastic resistance, to the impact of shocks of vehicles passing over the roadway, this elastic resistance preventing breaking, which is very 70 apt to occur with roadways which are very hard, such as those in which crushed or broken stone, as trap rock or pebbles and some hardening agent, is employed. Furthermore, in addition to its cheapness, substantially pure coal cinder has the added advantage that it may be obtained from innumerable sources and is available by most 75 municipalities as a waste product from their public buildings, which may be utilized in 80 road construction without any other material except a bituminous binder.

My improved roadway or pavement is, therefore, essentially one made of substantially pure coal cinder, and preferably sufficiently clinkered and free from fine ash so as not to disintegrate or grind up under the action of the roller by which the bed is compacted, and combined with a bituminous binder as hereinafter described. As an instance of such cinder, I would specify the 85 cinder ordinarily used for railroad ballast.

The accompanying drawing illustrates two ways of carrying out my invention. In this drawing, Figure 1 is a cross sectional 95 view showing the invention as embodied in a roadway having two layers of coal cinder and binder, and Fig. 2 a similar view showing the roadway as constructed with one layer.

Various methods may be employed for building the roadway of this cinder with a bituminous binder, depending somewhat on the character of road to be built and the probable amount of traffic which would be 105 carried thereover. A construction which has given satisfactory results, and which will preferably be used where the traffic is heavy, may be constructed as follows: The dirt or soil of the road to be constructed is 110

removed to the desired subgrade. On the dirt or soil is first laid a layer of cinder which is of a minimum thickness of two inches. The thickness of this first cinder layer may vary according to the character of the road desired, but I have found by experiment that six inches is usually sufficient. This cinder base is then rolled or compacted into a compact layer by means of any suitable roller of sufficient weight to effect the compacting but not sufficient to grind up the cinder, a roller of from five to ten tons usually being employed. This cinder layer having been rolled, a coating of a bituminous binder, such as heavy oil residuum of petroleum distillation is applied in any suitable manner, as by spraying from a tank under pressure or spreading by hand. This binder may be applied either in a cold state, or heated, the latter method, under certain circumstances, giving very good results, the binder being heated up to 75° to 100° F. This binder coating is allowed to percolate through the cinder, and with it forms a compact bed which at the same time may yield somewhat or have an elastic resistance to impact shocks. The binder may be used in any suitable quantities, depending on the density of the particular cinder used and on the thickness of the layer, the quantity varying from three fourths of a gallon to a gallon and a half per square yard. After the binder has sufficiently permeated the cinder, a second layer of substantially pure cinder of a thickness of from two to four inches is applied and rolled as was the first layer, and after the rolling there is applied a somewhat smaller amount of bituminous binder, the amount of the binder used in the second layer varying from one-quarter to three-quarters of a gallon per square yard, depending on the quality of cinder employed. For usual traffic conditions, a road-bed constructed as described will be of sufficient strength and durability and can be surfaced, as is usual, by spreading a thin coating of cinder or sand over the surface. After the second coating of binder has been applied, this cinder or sand is preferably rolled in. If, however, traffic is expected to be very heavy over the road, a third layer of cinder and binder similar to the second layer may be put on and then the finishing coating of cinder or sand applied. If, in constructing the road as described, after the cinder is rolled and before the application of the binder, the cinder should present large interstices, a thin layer of clay or sand may be spread over the layers to fill up these interstices before the binder is applied. This addition of clay or sand is, however, unnecessary, and may be omitted, as generally the cinder particles will so vary in size as to compact without having these undesirably large interstices.

If it is desired, and this is true particularly where light traffic is expected over the roads, such, for instance, as roads built away from main lines of travel; the road may be constructed with a somewhat thicker base of the cinder ballast and but one coating of the binder. Where the road is to be so constructed, it has been found that a layer of six to ten inches or more of cinder placed on the dirt subgrade and rolled as before described will give very good results. After this has been rolled there will be placed thereon a thinner layer of, say, two or three inches of cinder, which is then rolled and the binder applied as described, either hot or cold, and if desired then surfaced with a thin layer of cinder or sand. If desired, however, for light traffic roads, this second thinner layer of cinder may be omitted and the binder applied directly to the rolled cinder base. If desired, a curb of any suitable character may be provided on each side of the road to prevent the pavement from raveling, this curb being so laid that it is flush with the surface of the completed road and being left in position.

A roadway constructed as above described is one which may be built very cheaply because of the absence of the expensive trap rock or other stone heretofore considered necessary, and because its material is at the disposal of practically every town, or which can be obtained at a minimum of expense, and a roadway be produced which is durable for long periods. Furthermore, such a roadway, should any settling take place, or should the road be injured, may be very easily repaired by simply removing the bad spot, adding more cinder, a little binder, and rolling. Such a road is, therefore, very inexpensive to keep in repair. While the thicknesses of the cinder layers and the proportions per square yard of binder have been found in practice to be effective, it will be understood that different thicknesses of cinder layers may be employed and different proportions of binder used, depending on the particular character of road desired in any particular instance, and that the invention is not restricted to the thicknesses and proportions set forth.

What is claimed is:

1. A vehicle roadway or pavement having a foundation or ballasting rolled layer of substantially pure coal cinder, said cinder being of a size sufficient to withstand substantial disintegration or grinding up when rolled, a bituminous binder percolated through such rolled layer, and a superimposed rolled layer of cinder and a bituminous binder therefor, said layers being of sufficient thickness to resist the impact of the expected load.
2. A vehicle roadway or pavement comprising a rolled layer of substantially pure

- coal cinder of sufficient thickness to resist the impact of the expected load, said cinder being of a size sufficient to withstand substantial disintegration or grinding up 5 when rolled, and a bituminous binder applied to and percolated through the rolled layer.
3. The method of constructing a vehicle roadway or pavement which consists in preparing a dirt subgrade, putting down a layer of substantially pure coal cinder, rolling the cinder to compact it, applying a bituminous binder to the rolled layer so that it ~~may~~ percolate therethrough, superimposing a second layer of substantially pure coal cinder, rolling the second layer to compact it, and applying a bituminous binder to the second layer, the said layers being sufficiently thick to withstand the impact of the expected load. 20
4. The method of constructing a vehicle roadway or pavement, which consists in preparing a dirt subgrade, putting down a layer of substantially pure coal cinder, of sufficient thickness to withstand the impact 25 of the expected load, rolling the cinder to compact it, and adding a bituminous binder to the rolled cinder and allowing the binder to percolate through the layer. 25

In testimony whereof, I have hereunto set 30  
my hand.

BERNARD A. RUGE.